# EUROPEAN PATENT SPECIFICATION

(11) **EP 2 090 670 B1**
(45) Date of publication and mention of the grant of the patent: **25.05.2011**
(21) Application number: 07380339.7
(22) Date of filing: 05.12.2007
(51) Int. Cl.: C22C 33/08, G01N 25/06, C22C 37/04

(54) **Method for predicting spheroidisation degree in defined zones of spheroidal graphitic cast iron pieces**
Verfahren zur Vorhersage des Einformungsgrades in festgelegten Bereichen von Kugelgraphitgussteilen
Procédé pour la prédiction du degré de sphéroïdisation dans des zones définies de pièces de fer en fonte d'acier graphitique sphéroïdales

(43) Date of publication of application: 19.08.2009
(73) Proprietor: Casa Maristas Azterlan, 48200 Durango (ES)
(72) Inventor: Sertucha Pérez, Jon, 48200 Durango (Vizcaya) (ES); Suárez Creo, Ramón, 48200 Durango (Vizcaya) (ES)
(74) Representative: Gislon, Gabriele

(56) References cited:
- DE-A1- 2 919 625
- US-A- 3 670 558
- DIOSZEGI ET AL: "Inverse thermal analysis method to study solidification in cast iron" INTERNATIONAL JOURNAL OF CAST METALS RESEARCH, CAST METALS DEVELOPMENT, BIRMINGHAM, GB, vol. 17, no. 5, 1 January 2004 (2004-01-01), pages 311-318, XP009101329 ISSN: 1364-0461
- FRAS E ET AL: "Eutectic cell and nodule count in grey and nodular cast irons" MATERIALS SCIENCE AND TECHNOLOGY,, vol. 23, no. 9, 1 September 2007 (2007-09-01), pages 1109-1117, XP009101338 ISSN: 0267-0836
- SUN, X. J. ET AL: "Identification and evaluation of modification level for compacted graphite cast iron" JOURNAL OF MATERIALS PROCESSING TECHNOLOGY , 200(1-3), 471-480 CODEN: JMPTEF; ISSN: 0924-0136, 2008, XP002483725
- ZHU P ET AL: "Application of thermal analysis to predict the microstructure of cast iron" 4TH DECENNIAL INTERNATIONAL CONFERENCE ON SOLIDIFICATION PROCESSING, SHEFFIELD, UK, 7-10 JULY 1997,, 7 July 1997 (1997-07-07), pages 498-501, XP009101302 ISBN: 978-0-9522507-2-2

## Description

### Field of the Invention

The invention relates to a method predicting the degree of spheroidization in certain areas of spheroidal graphite casting cast pieces.

### State of the Art

The degree of spheroidization of a spheroidal graphite casting is a piece of data with great practical interest because it is a relevant indicator with regard to the mechanical behavior of the cast iron studied, and especially of its brittleness. The degree of spheroidization represents the number of graphite spheroids developed per mm² inside the material.

These graphite spheroids are developed during the cooling process, when carbon crystallizes in small spheroidal-shaped clusters in a uniform manner throughout the entire matrix. The determination of their number and concentration provides a clear idea of the metallurgical quality of the spheroidal graphite casting.

It is also known that the degree of spheroidization of the graphite of a molten metal, the size of the spheroids and the distribution thereof can be obtained from the analysis of the cooling curve of the mentioned molten metal.

In this sense, there are different patents relating to this topic, such as the following:
Patent JP60177116 mentions a method for accurately and quickly measuring the degree of spheroidization of the graphite in cast iron by means of using thermocouples and subsequent mathematical calculations, but it does not refer to the specific degree of nodulization of a specific area.
Patent W09400755 mentions a method for determining the graphite content of the casting by means of an ultrasonic system and the comparison of the results with a reference material. In this case, an average value is obtained and the influence of the shape of the piece is not observed either.
Patent US 6,604,016 discloses a new method for obtaining iron in which the graphite content can be accurately determined by means of controlling the cooling curve and the additives. This case is more of a production process and does not take into account the shape of the piece to be obtained.
Patent W09925888 shows another process for obtaining iron with spheroidal graphite, also by means of using cooling curves and modifying agents. It is an improvement of the previous method, but it still does not mention differentiated areas for the piece.
Patent AU651389B describes a process for obtaining ductile cast iron including the control of the cooling by means of using thermocouples and the correction of the composition by means of adding modifying agents to obtain the desired degree of nodularity. In this case, the degree of nodularity obtained in the different areas of the piece is not mentioned either and it is also a production process.
US3670558 discloses the technique of inverse thermal analysis applied to the study of solidification in cast iron allowing a common metallurgical background for samples solidifying at different cooling rates as they do when casting are placed in a cluster in a mould, performing relative measurements of the degree of spheroidization for each of the different samples in the mould.

In any case, none of these methods is suitable for calculating the degree of spheroidization of certain areas of the cast pieces, or in the case of processes, of achieving a casting of the piece in which a specific area thereof has the desired degree of spheroidization.

### General Description of the Invention

Different methods have traditionally been developed by means of thermal analysis technology due to the need to predict the mechanical behavior of different metal materials as accurately as possible. Thus, by means of pouring the liquid metal in a quik-cup (metallographic microstructural heat transfer model) and the analysis of its solidification process, essentially as regards its thermal components, it is possible to predict which degree of modularity that this metal will have.

This known methods orient the interpretation about the behavior of the material and its metallurgical quality level on a very important aspect, such as spheroidization. However, this method by no means takes into account the morphology of the pieces, their dimensions, modulus and other important considerations in the solidification process, therefore the obtained result is a generic piece of data independent of the piece.

In addition, what is really interesting to know from the industrial point of view, apart from knowing what will happen when a complete piece solidifies, is what happens in very specific areas which are especially problematic due to the thickness of such piece or to the fact that it will be highly stressed or because it can become a crack initiation point due to the fatigue load it will sustain.

In this situation, the generic determination of the number of spheroids that a liquid metal can develop, which is what the operating systems on the market currently offer, is completely insufficient.

The object of the present invention is to predict the spheroidization level which will be reached in a certain area of the previously selected spheroidal graphite cast piece which is located in a certain position of the cluster of pieces cast simultaneously into a mold. The concept of cooling rate, which is a determining factor in the nucleation and growth mechanisms of graphites, will be used in this development.

Traditional systems for determining the degree of spheroidization are based on the concept of Thermal Modulus. This parameter, associated to the cooling rate, is obtained as the ratio between the volume of the metal and the surfaces thereof which can evacuate heat and, in insulated system in which there are no other influencing elements modifying the cooling process and therefore the solidification process, it can be directly associated to the formation of graphite spheroids.

Studies conducted on test pieces (cylinders and cubes) of inoculated spheroidal graphite have allowed relating the graphite density (sph/mm²) at the geometric center thereof with the thermal modulus and with the metallurgical quality of the metal, represented by the spheroid density provided by the thermal analysis for the reference quik-cup (Figure 1).

The corresponding equation is therefore of the following type: $No . of spheroids = f \left(M, {N}_{at}\right)$
where the number of spheroids is given in sph/mm², M is the thermal modulus (cm) and Nₐₜ is the prediction provided by the thermal analysis for the quik-cup in sph/mm²

However, the conditions of the real pieces in casting processes do not coincide with those of an insulated system, it is therefore necessary to introduce and develop the concept of a new parameter taking into account not only traditional determining factors, but also the morphology of the piece to be cast and all the particular elements affecting the heat evacuation in each of its parts. At this point, the Inverse Modulus is defined as the modulus to which the graphitization level shown by the piece in a certain area corresponds. In other words, it is real capacity that a certain area has for evacuating heat energy. The method of the invention is given in the claim.

This Inverse Modulus, associated to a specific area of the piece, is calculated from the real number of spheroids of that area (metallographically controlled) and from the prediction obtained by means of thermal analysis (Nₐₜ) (Figure 2).

The main advantage that this system will allow obtaining is the accurate knowledge of the degree of spheroidization, and thus of the properties of a certain area of a piece located in a certain place of the cluster of pieces that are simultaneously cast in a mold. This knowledge will allow defining its behavior with greater reliability, thus assuring the structural integrity of the system or structure and facilitating its sizing.

The main usefulness of the method is based on the fact that subsequent simulations and predictions on the same cluster of pieces using the inverse modulus in each simulation this time will give a much more accurate estimation than when traditional means are used. Thus, upon any variation of the casting conditions, a variation of the temperature of the molten material, for example, the simulation systems will predict the degree of spheroidization which will be obtained in a much more accurate manner, allowing the caster to introduce the relevant corrective measures.

### Brief Description of the Drawings

Figure 1 shows the graphic representation of the cooling curve according to time.
Figure 2 shows the methodology followed in the development for calculating the Inverse Modulus based on the thermal analysis and the metallographic study.
Figure 3 shows the fork used in practical case 1.
Figure 4 shows the fork used in practical case 2.

### Detailed Description of Particular Embodiments

Two examples for applying the method for predicting the degree of spheroidization in defined areas of spheroidal graphite cast pieces according to their inverse modulus are included below.

### Case 1: It is a vehicle brake fork in which four areas are differentiated: (Figure 3)

1.- The areas must first be differentiated:
   Area 1: Mid part of the lower thin arch
   Area 2: Mid part of the upper thick arch
   Area 3: Left hub adjacent to the upper arch
   Area 4: Right hub adjacent to the upper arch
2.- In each of the previous areas, the thermal modulus is calculated by means of the classic methodology, obtaining the following results:
   Area 1: Mt = 0.28 cm
   Area 2: Mt = 0.57 cm
   Area 3: Mt = 0.62 cm
   Area 4: Mt = 0.62 cm
3.- The generic number of spheroids is predicted by means of quik-cup according to the established metallurgical quality and the thermal modulus.
   Area 1: Nsph(gen) = 350 sph/mm²
   Area 2: Nsph(gen) = 300 sph/mm²
   Area 3: Nsph(gen) = 290 sph/mm²
   Area 4: Nsph (gen) = 290 sph/mm²
4.- Determination of the real number of spheroids in the target area by means of metallographic analysis
   Area 1: Nsph(met) = 435 sph/mm²
   Area 2: Nsph(met) = 260 sph/mm²
   Area 3: Nsph(met) = 242 sph/mm²
   Area 4: Nsph(met) = 242 sph/mM²
5.- Calculation of the inverse modulus according to the metallurgical quality and the number of spheroids of the piece obtained in the previous step
   Area 1: Mi = 0.28 cm
   Area 2: Mi = 0.60 cm
   Area 3: Mi = 0.67 cm
   Area 4: Mi = 0.67 cm
      This value is calculated for different qualities, i.e. for different spheroid density values, therefore the value obtained at the end is an average value of those obtained in all the tests. It can generally be stated that there is not much difference between the obtained values.
6.- Prediction of the number of spheroids according to the inverse modulus
   In this step the number of spheroids is calculated using the average value of the inverse modulus calculated in the previous section.

### Case 2: A brake fork different to the previous one is again used to start from.

1.- The areas must first be differentiated; four areas in this case (Figure 4)
2.- In each of the previous areas, the thermal modulus is calculated by means of the classic methodology, obtaining the following results:
   Area 1: Mt = 0.28 cm
   Area 2: Mt = 0.37 cm
   Area 3: Mt = 0.71 cm
   Area 4: Mt = 0.71 cm
3.- The generic number of spheroids is predicted by means of quik-cup according to the established metallurgical quality and the thermal modulus.
4.- The real number of spheroids in the target area is determined by means of metallographic analysis
   Area 1: Nsph(met) = 432 sph/mm²
   Area 2: Nsph(met) = 319 sph/mm²
   Area 3: Nsph(met) = 229 sph/mm²
   Area 4: Nsph(met) = 229 sph/mm²
5.- The inverse modulus is calculated according to the metallurgical quality and the number of spheroids of the piece obtained in the previous step
   Area 1: Mi = 0.30 cm
   Area 2: Mi = 0.47 cm
   Area 3: Mi = 0.77 cm
   Area 4: Mi = 0.77 cm
      This value is calculated for different qualities, i.e. for different spheroid density values, therefore the value obtained at the end is an average value of those obtained in all the tests. It can generally be stated that there is not much difference between the obtained values.
6.- Finally, the number of spheroids is predicted according to the inverse modulus, using the average value of the inverse modulus calculated in the previous section.

## Claims

1. A method for predicting the degree of spheroidization of spheroidal graphite cast pieces, suitable for specifically predicting the degree of spheroidization in any specific area of any piece located in a cluster of pieces that are simultaneously cast in a mold, said prediction being carried out according to the specific solidification conditions of the cluster and according to the specific inverse modulus of the area of the piece in question, said inverse modulus being determined from conventional predictions of the degree of spheroidization by thermal analysis and actual measurements of the degree of spheroidization in previously cast pieces, wherein said method, once certain areas have been differentiated in the piece, comprises:
a) determining the thermal modulus of each area of the piece by means of conventional methodology,
b) predicting the number of spheroids in each area of the piece by means of conventional thermal analysis tools based on the thermal modulus of each area, **characterized in that** it further comprises:
c) determining the actual number of spheroids by means of direct metallographic analysis of each area,
d) calculating said inverse modulus according to the metallurgical quality by metallographic techniques, and
e) predicting the number of spheroids in each area of the piece by means of conventional thermal analysis tools based on the inverse modulus of each area which has been calculated from the real number of spheroids of that area, metallographically measured and from the prediction obtained by means of the conventional thermal analysis.

## Patentansprüche

1. Verfahren zur Vorhersage des Sphäroidisierungsgrads von Kugelgraphit-Gussteilen, welches dazu geeignet ist, gezielt den Sphäroidisierungsgrad in jedem spezifischen Bereich von jedem Teil vorherzusagen, das sich in einer Gruppe aus Teilen befindet, welche gleichzeitig in einer Form gegossen werden, wobei die genannte Vorhersage gemäß den spezifischen Erstarrungsbedingungen der Gruppe und gemäß dem spezifischen inversen Modulus von dem Bereich des betreffenden Teils durchgeführt wird, wobei der genannte inverse Modulus aus herkömmlichen Vorhersagen des Sphäroidisierungsgrads durch Thermoanalyse und tatsächlichen Messungen des Sphäroidisierungsgrads in vorher gegossenen Teilen bestimmt wird, wobei das genannte Verfahren, nachdem bestimmte Bereiche in dem Teil differenziert worden sind, Folgendes umfasst:
a) Bestimmen des Wärmemoduls von jedem Bereich des Teils mittels herkömmlicher Methodik,
b) Vorhersagen der Anzahl von Sphäroiden in jedem Bereich des Teils mittels herkömmlicher Mittel für Thermoanalyse, basierend auf dem Wärmemodul von jedem Bereich, **dadurch gekennzeichnet, dass** es zusätzlich Folgendes umfasst:
c) Bestimmen der tatsächlichen Anzahl von Sphäroiden mittels direkter metallographischer Analyse von jedem Bereich,
d) Berechnen des genannten inversen Modulus gemäß der metallographischen Qualität durch metallographische Techniken, und
e) Vorhersagen der Anzahl von Sphäroiden in jedem Bereich des Teils mittels herkömmlicher Mittel für Thermoanalyse, basierend auf dem inversen Modulus von jedem Bereich, der aus der, metallographisch gemessenen, tatsächlichen Anzahl von Sphäroiden in diesem Bereich berechnet worden ist und aus der durch herkömmliche Thermoanalyse erreichten Vorhersage.

## Revendications

1. Une méthode pour prédire le degré de sphéroïdisation de pièces fondues en graphite, sphéroïdales, appropriée pour prédire spécifiquement le degré de sphéroïdisation dans toute région spécifique de toute pièce située dans un groupe de pièces qui sont simultanément fondues dans un moule, cette prédiction étant effectuée dans des conditions de solidification spécifique du groupe et conformément au module inverse spécifique de la région de la pièce en question, ce module inverse étant déterminé à partir de prédictions conventionnelles du degré de sphéroïdisation par l'analyse thermique et les mesures réelles du degré de sphéroïdisation dans des pièces préalablement fondues, où cette méthode, lorsque certaines régions ont été différenciées dans la pièce, comporte:
a) la détermination du module thermique de chaque région de la pièce au moyen de la méthodologie conventionnelle,
b) la prédiction du nombre de sphéroïdes dans chaque région de la pièce au moyen d'outils d'analyse thermique conventionnels basée sur le module thermique de chaque région, **caractérisée en ce que** de plus elle comporte :
c) la détermination du nombre réel de sphéroïdes au moyen de l'analyse métallographique directe de chaque région,
d) le calcul de ce module inverse conformément à la qualité métallurgique au moyen de techniques métallographiques, et
e) la prédiction du nombre de sphéroïdes dans chaque région de la pièce au moyen d'outils d'analyse thermique conventionnels basée sur le module inverse de chaque région qui a été calculée à partir du nombre réel de sphéroïdes de cette région, métallographiquement mesuré et de la prédiction obtenue au moyen de l'analyse thermique conventionnelle.
